

# UNITED STATES PATENT OFFICE.

LINDON W. BATES, OF MOUNT LEBANON, NEW YORK.

## FUEL AND METHOD OF PRODUCING SAME.

1,382,457.

Specification of Letters Patent. Patented June 21, 1921.

No Drawing. Original application filed August 5, 1919, Serial No. 315,497. Divided and this application filed May 17, 1920. Serial No. 381,826.

To all whom it may concern:

Be it known that I, LINDON W. BATES, a citizen of the United States, residing at Mount Lebanon, in the county of Columbia 5 and State of New York, have invented certain new and useful Improvements in Fuels and Methods of Producing Same, of which the following is a specification.

This invention pertains to a mobile fuel 10 in which immiscible liquid hydrocarbons are stabilized with the aid of particles of solid carbonaceous substance. Many liquid combustibles are miscible with others, but several important classes of such fuels are 15 refractory to stable combination. Thus, there has been an especial desire to obtain "a fuel oil suitable for admiralty uses made of admixture of dehydrated coal tar with mineral petroleum oils." Oils do not ordinarily dis- 20 solve or emulsify with such tars and more or less rapid separation or uncontrolled stratification has heretofore prevented their combined use as mobile or liquid fuel. The same condition prevails in the case of other 25 liquids.

In my copending application, Serial No. 315,497, filed on August 5th, 1919, of which this is a division, the question of stability was fully considered in the light of Stokes's 30 law for the terminal velocity of fall of a spherical body in a liquid. Droplets of one liquid in another liquid with which the first is immiscible or is partially miscible only, disclose somewhat similar stability characteristics. There are, however, lesser deviations from Stokes's law as the droplets are 35 nearly spherical, unless the volume of the disperse phase exceeds 74% of that of the total liquid. Liquid dispersed droplets are 40 stable in a liquid medium when they are of molecular size or when they are sufficiently within colloidal limits. In the case of an oil emulsion in water the oil droplets do not separate from the water until they are above 45 one micron in size. Stable emulsions may be formed of one part of oil in ten thousand parts of water. Suspension-sized droplets are unstable.

With reference to stabilizing two or more 50 immiscible or partially miscible liquid hydrocarbons in each other, the interesting scientific fact has been disclosed that the presence of a considerable percentage by weight of pulverized carbonaceous sub- 55 stance, without reduction to colloidal limits

in size, has the effect, when the components are duly mixed, of stabilizing them. In so doing the particles are themselves stabilized in the liquid. In such a composite there is no need of either a protective agent or a 60 peptizing agent as defined in my copending application. In fact one may omit these agents and still obtain adequate stability. Substances which greatly lower the surface tension of liquid against liquid are adsorbed 65 by these. In a mixture of oil, tar and pulverized coal, for example, the stabilization effect of the coal and tar upon each other is to a certain extent reciprocal. That is, the coal and the tar together in oil may be stabilized more readily than either alone. 70

In relation to stabilizing such immiscible liquid hydrocarbons with the aid of pulverized carbonaceous substances the percentage of necessary particles varies with the 75 nature and relative amounts of liquid hydrocarbons. In general, up to about 20% by weight, of total fuel, of a heavy tar may be stabilized in oil, and larger amounts of the lighter varieties. From 10% to 30% of 80 particles will be necessary. From experience, the greatest amount of tar may be stabilized in pressure still oil with the aid of coal. An adequately stable composite may be made, for example, consisting by 85 weight of about 50% pressure still oil, 20% coke-oven by-product tar, and 30% pulverized coal. If an oil such as that from Texas complying with Navy standards is used the proportion of coal or other carbonaceous substance to tar has to be increased and the proportion of coal and tar to oil has to be decreased. With a paraffin base Navy fuel oil of low viscosity, less tar than 20% and less coal than 30% can be 90 adequately stabilized together in this manner. If a small amount of protective agent is added to the mixture, the highest amount of tar may be stabilized in oil with the aid of coal or other such carbonaceous particles. 95 So also the aid of peptization may be invoked, to supplement the ability of pulverized coal to artificially induce the stability of itself and tar as a suspension in oil. 100

It is not claimed herein that all immiscible 105 liquid hydrocarbons may be stabilized with the aid of particles of solids for fuel purposes, but it has been found that such liquid combustibles as mineral oils with coal tars are readily so combined. Liquid hydrocar- 110

bons of analogous nature and characteristics, whether mineral, animal or vegetable, are also susceptible to such combination. By the term "immiscible" is meant substantial non-miscibility, as there is nearly always some miscibility between even very dissimilar liquids.

A product heavier than water is sought so that it may be stored under a water seal 10 for fireproofing purposes. Since greater percentages of particles than 10% are usually required for stability, the product enjoys a specific gravity above unity. The particles and droplets themselves remain 15 for the most part well above the colloid in size. By the term "mobile" is meant a fuel sufficiently fluid to allow its atomization through burners as liquid fuel is now used. By "stable" is meant non-separation of the 20 components sufficient in degree and duration to enable such use of the fuel without resort to continuous agitation or stirring to maintain suspension. Furthermore the stability must be of such a character that there 25 is no undue separation either at normal temperature around 70° F. or at low temperatures in storage, or at high temperatures, up to 250° F., in the preheater. Simple non-separation at normal temperature or 30 thereabouts is not sufficient if stability does not duly persist when the fuel is preheated preparatory to atomization or conveyance.

By "protective agent" is meant a substance which acts to stabilize in the fashion 35 of the lime-rosin grease described in my said copending application. The action is conceived to be somewhat analogous to that of a protective colloid upon colloids. On the other hand, by "peptizing agent" is meant 40 a substance which acts to peptize and stabilize in the fashion of coal distillates, such as creosote, under the heat treatment described fully in the application aforesaid. The term "peptization" is used to signify di- 45 gestion of the particles, that is to say, a partial reduction in size by dissolving and also a spongifying, pitting and cavitating of the particles which promotes stability.

The carbonaceous particles used in the present process should be reduced by pulverization or otherwise to a size such that about 50 85% would pass a 200-mesh screen. No suitable substances of such requisite fineness are found in their natural state. Artificial 55 reduction is therefore essential. By the term "pulverized" is meant, therefore, artificial reduction to the size mentioned, so that the relative stability may be obtained.

The liquid dispersion medium need not 60 be of low viscosity, since a heavy oil or tar may be so used. Likewise, the immiscible liquid which it is desired to combine therewith need not be a heavy liquid. If the dispersion medium is heavy in regard to viscosity or fluidity, the immiscible liquid

added thereto is preferably of low viscosity, so that the viscosity of the composite will be moderate or low. A product of moderate or low viscosity is sought as such fuels atomize more readily than those of high viscosity. Thus if a Mexican petroleum residual oil is selected as the dispersion medium, the liquid added thereto should be of low viscosity, such as water gas tar. If light pressure still oil or tar is the base, it 75 is entirely proper to combine therewith a heavy coal tar. In other words, the present method does not rely solely or chiefly upon an increase in the viscosity of the medium to promote stability. It is indeed true that 80 the very use of particles of coal tends to produce a composite of less fluidity than that of the liquids used therein, but a stable composite may be made of moderate viscosity insufficient *per se* to prevent sedimentation or separation. In fact the lower the viscosity of the composite, consistent with stability, the superior the fuel for use as liquid combustible. While an increase in viscosity may be resorted to or may occur 90 as a collateral means of promoting stability, it is not featured herein, and the present method is independent thereof. As heretofore remarked, stability must persist sufficiently to allow atomization without congestion in the pipes when the viscosity is 95 reduced by heat.

The mixing treatment necessary to obtain the desired stability consists in mechanical blending of the ingredients, with or without heat treatment in the manufacture. By mixing the components for a few minutes in an ordinary paint, ball or tube mill or other suitable mixing machine, in which no abnormal pressure or high speed need be used, 105 the homogeneous quality is well obtained. The desired homogeneity may also be promoted by pulverizing the carbonaceous substance initially in the liquid hydrocarbons, using a similar type of apparatus, instead 110 of mixing the components after the carbonaceous substance has already been pulverized. Furthermore, proper diffusion of the particles through the liquid and association therewith, and hence adequate homogeneity, 115 may be obtained by giving the composite a heat or a heat and mixing treatment, causing such a movement of the components as tends to mix and unite them thoroughly. If the heat is raised to between 65° C. and 95° C. the homogeneity will become satisfactory. The duration of the mixing treatment varies with the components and with 120 the stability desired. The introduction of new components and the withdrawal of already mixed components may take place simultaneously in a continuous process, or the "batch" system may be employed. The dispersion medium may be a single liquid or a blend. The immiscible liquid

added thereto may also be of one variety or of several. The particles of solids may be coals, cokes, peats, pitches, or lignites, or a mixture of these.

The present stabilization process should be carefully distinguished from stabilization by peptization described in my copending application. In the present case, it is not necessary to bring into operation the peptization reaction to stabilize, even if a liquid having peptizing capacities is present in the composite. Thus non-peptizing cokes will serve the stabilizing purpose. Heat is usually required to induce peptization as the capacity is so to speak latent, but there are a few coal derivatives which are active peptizers at normal temperature if time is allowed for them to operate upon the particles. Some of the tars immiscible with oils possess peptizing qualities, either active or latent. The present method will stabilize whether aided by actual peptization or not. If the components include a peptizer and the carbonaceous particles are susceptible of peptization and heat is employed in the manufacture or long storage is allowed, partial or proper peptization for stability may eventuate, thus collaborating with the present method in attaining the stability result. The present method is independent of peptization and no sole or principal reliance upon it is herein placed.

This application is a division of my application Serial No. 315,497, filed August 5, 1919.

Having thus described the nature of my invention, what I claim is:

1. A stable mobile fuel containing particles of solid carbonaceous substance and a plurality of incompletely miscible liquid hydrocarbons.

2. A mobile atomizable fuel of relative stability, heavier than water, consisting of particles of artificially pulverized solid carbonaceous substance and a plurality of substantially immiscible liquid hydrocarbons.

3. A mobile atomizable fuel of relative stability, heavier than water, consisting of particles of artificially pulverized solid carbonaceous substance, with oil and tar which are substantially immiscible together.

4. A mobile atomizable fuel heavier than water, consisting essentially of mineral oil, tar substantially immiscible therewith, and an amount of artificially pulverized solid 55 carbonaceous substance which serves to stabilize the tar and the carbonaceous substance in the oil.

5. A mobile atomizable fuel heavier than water, which consists approximately by 60 weight of 60% mineral oil, 15% dehydrated coal tar, and 25% artificially pulverized solid carbonaceous substance.

6. That method of combining as a relatively stable atomizable mobile fuel two or 65 more substantially immiscible liquid hydrocarbons, which consists essentially in homogenizing therewith particles of artificially pulverized solid carbonaceous substance.

7. That method of producing an atomizable mobile fuel of relative stability, which consists in adding to a plurality of substantially immiscible liquid hydrocarbons particles of artificially reduced solid carbonaceous substance in an amount which raises 75 the specific gravity of the composite above that of water, and homogenizing the components with the addition of substance having stabilizing qualities.

8. That method of producing an atomizable mobile fuel of relative stability, which comprises adding to a plurality of substantially immiscible liquid hydrocarbons particles of artificially reduced solid carbonaceous substance in an amount which raises 85 the specific gravity of the composite above that of water, homogenizing the components and peptizing the particles.

9. That method of producing an atomizable mobile fuel of moderate viscosity and 90 relative stability, heavier than water, which comprises taking an oil of high viscosity, adding thereto a tar of low viscosity substantially immiscible therewith and an amount of particles of artificially pulverized 95 solid carbonaceous substance sufficient to raise the specific gravity of the composite above that of water, and homogenizing the components until the composite is stabilized.

In testimony whereof I have signed my 100 name to this specification.

LINDON W. BATES.